

## UNITED STATES PATENT OFFICE

2,069,303

## PROCESS OF TREATING TEXTILE MATERIALS AND PRODUCT THEREOF

Camille Dreyfus, New York, N. Y., and William Whitehead, Cumberland, Md., assignors to Celanese Corporation of America, a corporation of Delaware

No Drawing. Application November 7, 1931,  
Serial No. 573,718. Renewed June 26, 1936

14 Claims. (Cl. 91—68)

This invention relates to the treatment of textile materials such as yarns, filaments, fabrics and the like and relates more particularly to the treatment of textile materials containing organic derivatives of cellulose in order to improve their textile properties.

An object of our invention is to improve the properties of textile materials by incorporating therein a lower monohydric alcohol ester of a higher fatty acid. Other objects of this invention will appear from the following detailed description.

Often it is desirable to increase certain physical properties of textile materials such as wearing properties or scroop, or diminish undesirable properties such as tendency to slip, ladder, etc. We have found that if a lower monohydric alcohol ester of a higher fatty acid is incorporated in such textile material, particularly one containing cellulose acetate or other organic derivative of cellulose, such objects are attained.

In accordance with our invention we incorporate in a textile material, particularly one containing an organic derivative of cellulose, a lower monohydric alcohol ester of a higher fatty acid.

The textile material to be treated in accordance with this invention may be in the form of yarns, filaments, artificial bristles or straw, or it may be a woven, knitted or netted fabric containing such yarns, filaments, straw or bristles.

The textile material treated by this invention preferably contains organic derivatives of cellulose such as organic esters of cellulose and cellulose ethers. Examples of such organic esters of cellulose are cellulose acetate, cellulose formate, cellulose butyrate, while examples of cellulose ethers are ethyl cellulose, methyl cellulose and benzyl cellulose. However the textile material may be made of other fibres such as natural silk, reconstituted cellulose, cotton, flax, wool, or it may be a mixed material containing such fibres and filaments or yarns of organic derivatives of cellulose.

While we prefer to employ methylstearate, other lower monohydric alcohol esters of a higher fatty acid, particularly such an ester of a higher saturated fatty acid may be employed. Examples of these, besides methyl stearate, are ethyl stearate, propyl stearate, butyl stearate, methyl palmitate, ethyl palmitate, propyl palmitate and butyl palmitate. However, the esters of unsaturated fatty acids such as the methyl, ethyl, propyl or butyl ester of oleic acid may also be employed in our invention.

In one form of our invention, the methyl stear-

ate or other ester of the fatty acid may be applied as a finish to the yarn at the spinning cabinet from which it is formed, or while it is otherwise in transit to a packaging device, by means of wicks, rolls or other furnishing devices. If desired the yarns may be treated in the form of hanks. The methyl stearate and like fatty acid ester may be applied to the yarn in conjunction with other lubricants such as olive oil, diethylene glycol, ethyl oxybutyrate or mixtures of two or more of these.

In another form of our invention, the methyl stearate and like fatty acid ester may be applied to a woven, knitted or netted fabric by dipping, spraying and the like.

In still another form of our invention, the monohydric alcohol ester of the fatty acid may be added to a spinning dope, such as a solution of cellulose acetate in acetone, from which the yarns, filaments and the like may be formed by extrusion into a drying evaporating medium or into a liquid coagulating bath.

The methyl stearate and like ester may be applied to the yarn or fabric either in concentrated or pure form, or dissolved in a suitable solvent therefor or in the form of an emulsion. Thus methyl stearate may be applied while dissolved in benzol to form solutions of 0.1 to 25% concentration. The methyl stearate may be emulsified in aqueous solutions of soaps such as olive oil soap or triethanolamine oleate and the like to form emulsions of the same concentration. The methyl stearate or like ester is applied in amounts from 0.25 to 5%, preferably 0.5 to 2%, of the weight of the yarn or fabric.

Yarns, filaments, straw or bristles when treated in accordance with this invention have less tendency to slip than untreated material, and therefore firmer yarn packages, such as pirns, cones, bobbins, cops, etc., may be formed from them.

Fabrics when treated in accordance with this invention, or when made from yarn treated in accordance with this invention, have many desirable properties. Such fabric has greater wearing properties, as much as 25% or more, than untreated fabric as shown by a rubbing test with the Wyzenbeek & Staff precision wear test meter. Such woven fabric has less tendency to slip and such knitted fabric has less tendency to ladder than untreated fabric. Moreover such fabric does not tend to ravel as readily at cut edges as do untreated fabrics. Another further important advantage of this invention is that fabric containing the methyl stearate or like ester has an enormously increased scroop, which is of im-

portance for taffeta and like woven fabrics where scoop is desired.

In order further to illustrate our invention, but without being limited, the following specific 5 example is given.

*Example*

A fabric of taffeta weave consisting wholly of 10 yarns of cellulose acetate is impregnated with a solution of methyl stearate in benzene having a concentration of 0.5 to 2%, or an emulsion of methyl stearate in a solution of olive oil soap having a like concentration. The amount of liquor that the fabric is permitted to take up is 15 such that the amount of methyl stearate remaining on the fabric is from 0.5 to 2% of the weight of the fabric. The fabric is then dried, either at atmospheric temperatures or at elevated temperatures, in a suitable manner.

20 The fabric so treated shows an increase of over 25% in wearing properties as compared by friction tests with the untreated fabric, has an enormously increased scoop, and does not tend to slip or ravel as readily as the untreated fabric.

25 It is to be understood that the foregoing detailed description is given merely by way of illustration and that many variations may be made therein without departing from the spirit of our invention.

30 Having described our invention, what we desire to secure by Letters Patent is:

1. Process for the production of textile materials of improved properties, which comprises applying to textile materials, containing an organic derivative of cellulose, a preparation containing a water-insoluble lower monohydric alcohol ester of a higher fatty acid and drying the textile materials while retaining said ester therein.

2. Process for the production of textile materials of improved properties, which comprises applying to textile materials, containing cellulose acetate, a preparation containing a water-insoluble lower monohydric alcohol ester of a higher fatty acid and drying the textile materials while retaining said ester therein.

45 3. Process for the production of textile materials of improved properties, which comprises applying to textile materials, containing cellulose acetate, a non-aqueous preparation containing a water-insoluble lower monohydric alcohol ester of a higher fatty acid and drying the textile materials while retaining said ester therein.

40 4. Process for the production of textile materials of improved properties, which comprises applying to textile materials, containing cellulose acetate, an aqueous preparation containing a water-insoluble lower monohydric alcohol ester of a higher fatty acid and drying the textile materials while retaining said ester therein.

50 5. Process for the production of textile materials of improved properties, which comprises applying to textile materials, containing an or-

ganic derivative of cellulose, a preparation containing a lower monohydric alcohol ester of stearic acid and drying the textile materials while retaining said ester therein.

6. Process for the production of textile materials of improved properties, which comprises applying to textile materials, containing an organic derivative of cellulose, a preparation containing a lower monohydric alcohol ester of palmitic acid and drying the textile materials while retaining 10 said ester therein.

7. Process for the production of textile materials of improved properties, which comprises applying to textile materials, containing an organic derivative of cellulose, a preparation containing 15 methyl stearate and drying the textile materials while retaining said methyl stearate therein.

8. Process for the production of yarn of improved properties, which comprises applying to yarn containing an organic derivative of cellulose, prior to its formation into a fabric, a preparation containing a water-insoluble lower monohydric alcohol ester of a higher fatty acid and drying said yarn while retaining 20 said ester therein.

25 9. Process for the production of a fabric of improved properties, which comprises applying to a fabric, containing yarns of organic derivatives of cellulose, a preparation containing a water-insoluble lower monohydric alcohol ester of a 30 higher fatty acid and drying said fabric while retaining said ester therein.

10. Fabric comprising yarns of organic derivatives of cellulose having a water-insoluble lower monohydric alcohol ester of a higher fatty acid 35 incorporated therein in amount of 0.25 to 5%, whereby its wearing property is enhanced.

11. Fabric comprising yarns of cellulose acetate having a water-insoluble lower monohydric alcohol ester of a higher fatty acid incorporated 40 therein 1:1 amount of 0.25 to 5%, whereby its wearing property is enhanced.

12. Fabric comprising yarns of cellulose acetate having methyl stearate incorporated therein in amount of 0.25 to 5%, whereby its wearing 45 property is enhanced.

13. Textile materials of improved properties containing an organic derivative of cellulose, said materials having incorporated therein a water-insoluble lower monohydric alcohol ester of a 50 higher fatty acid in amount of 0.25 to 5%, and being substantially free from water in excess of that retained by the materials when exposed to the atmosphere.

14. Textile materials of improved properties 55 containing cellulose acetate, said materials having incorporated therein methyl stearate in amount of 0.25 to 5% and being substantially free from water in excess of that retained by the materials when exposed to the atmosphere.

CAMILLE DREYFUS.

WILLIAM WHITEHEAD.